

# UNITED STATES PATENT OFFICE.

WALTER R. BARDSLEY, OF PHILADELPHIA, PENNSYLVANIA.

## PROCESS FOR MAKING DIE-PLATES.

1,157,493.

Specification of Letters Patent. Patented Oct. 19, 1915.

No Drawing.

Application filed January 27, 1915. Serial No. 4,765.

To all whom it may concern:

Be it known that I, WALTER R. BARDSLEY, a citizen of the United States, residing at Philadelphia, in the county of Philadelphia and State of Pennsylvania, have invented 5 certain new and useful Improvements in Processes for Making Die-Plates; and I do hereby declare the following to be a full, clear, and exact description of the invention, such as will enable others skilled in the art to which it appertains to make and use the same, reference being had to the accompanying drawings, and to the letters and figures of reference marked thereon, which 10 form a part of this specification.

This invention relates to certain new and useful process for making a die or matrix of zinc, copper or other metal, the same to be used for embossing of printing plates so 15 that said printing plates may be used without an overlay or other "make-ready."

To this end and to such others as the invention may pertain, the same consists of the steps comprising the process hereinafter 20 described.

1. In carrying out my process, I first polish and clean the sheet of metal until it is entirely free from grease.

2. The metal surface thus cleansed is then 25 coated with sensitized fish glue or albumen solution, such as is commonly used in connection with the photo-engraving processes and is then dried in a subdued light.

3. The impression is then made upon the 30 sensitized metal plate, with any suitable full-bodied greasy ink, of the printing plate it is desired to treat or emboss.

4. After this step of the process, to the 35 surface of the plate is applied a fine opaque powder, such for instance as dragon's blood or the like. The excess powder upon the surface is then brushed away by a soft camel's hair brush or a piece of fine cotton wool.

45 5. The plate is then exposed to either a natural or artificial light for a length of time sufficient to make the sensitized solution on the plate insoluble in water.

6. The plate is then washed with turpentine, benzole, benzin or other suitable solvent 50 for the purpose of removing the ink and powder from the plate, care being taken not to scratch the surface.

7. The surface then is treated by the use 55 of a soft roller with a thin coating of good quality etching or lithograph transfer ink,

care being taken to insure an even spreading of the coating over the entire surface of the plate.

8. The plate is then immersed in a tray 60 of clear water and rubbed gently with a piece of cotton wool until the portions that have not been exposed to the light are washed clean. The portions of the plate covered by the ink mentioned in the third stage of 65 the operation will be found to be unaffected by the light and consequently will be soluble in water.

9. The plate is then powdered with dragon's blood or other suitable etching powder 70 and is heated slowly until the powder melts and the back of the plate is then coated with a suitable acid resist, such as shellac or asphaltum.

10. The plate is then placed in a tray containing acid, suitable for the metal used, and is etched from 1/1000 to 2/1000 of an 75 inch to any depth desired. After the etching, the surface of the plate is cleansed by the use of a proper solvent, such as benzole, 80 turpentine or caustic potash, which latter may be used when the coating is particularly hard to remove. Then, after drying, the portions of the plate which are of satisfactory depth are painted with an acid resist, 85 such as asphaltum and the plate is then etched to another degree. This painting and etching is alternately repeated until the necessary number of steps is acquired, usually three or four. 90

During the carrying out of my process from the second to the seventh step of the operation, care should be taken that no moisture other than that specified comes in contact with the plate. During the second, 95 third, fourth, sixth and seventh steps of the operation, the plate must be kept in a subdued light. It is necessary that the back of the plate should be constantly protected by a coating of shellac or asphaltum against 100 the action of acid. The metal sheets used in the process must necessarily be of even thickness throughout, ordinarily from 10/1000 to 18/1000 of an inch having been found satisfactory.

In the carrying out of the process, the 105 third and fourth steps of the process may be modified as, for instance, an impression may be taken, from the printing plate it is desired to emboss, upon a sheet of suitable 110 paper, using an abundance of ink. A transfer from this proof on paper can be made

to a sheet of transparent material such, for instance, as celluloid, gelatin or glass. The transfer is then dusted with a suitable fine opaque powder, such as bronze, dragon's blood, etc., for the purpose of making the image more dense so that it may be used as a photographic negative. The transfer is then brought in contact with the sensitized metal plate described in the second 10 operation and may be placed in a photographic frame, after which it may be treated to the steps described in the fifth operation. When this alternative operation is used, the sixth operation will be unnecessary.

15 Having thus described my invention, what I claim to be new and desire to secure by Letters Patent is:—

20 A method of making a metallic die for use in embossing, consisting in cleansing a metallic surface, coating the same with an albumen solution and drying the same in a subdued light and upon which an impression

is made by the use of ink, after which to the surface of the plate is applied a fine opaque powder, afterward exposing the 2 plate to light a sufficient length of time to cause the sensitized solution to the plate to be insoluble in water, afterward washing the plate with a solvent to remove the ink and powder from the plate, then treating 30 the surface of the plate with a coating of lithograph transfer ink, immersing the plate in liquid, washing off the portions which have not been exposed to the light, afterward applying suitable etching powder to 35 the surface and heating until the powder melts, and afterward etching the plate.

In testimony whereof I hereunto affix my signature in presence of two witnesses.

WALTER R. BARDSLEY.

Witnesses:

JOSEPH S. LORD,  
R. M. REMICK.

Copies of this patent may be obtained for five cents each, by addressing the "Commissioner of Patents, Washington, D. C."